

## UNITED STATES PATENT OFFICE

2,371,573

## PROCESS OF MAKING RAMIE YARN

Mark Sabner, London, W.1, England

No Drawing. Application June 25, 1940, Serial No.  
342,362. In Great Britain June 30, 1939

2 Claims. (Cl. 28—75)

This invention relates to ramie yarn and articles, especially hose pipes such as are employed by the fire-fighting services, and other material made of relatively fine count yarn, especially water-impervious material, woven therefrom, and to processes for producing the same.

Such articles as heretofore produced have a harsh "feel," cannot be woven very closely and have not the strength which should be expected in view of the stronger character of ramie fibre, as compared with flax, for example. The ramie yarn from which such articles have been woven has been spun wet.

Unlined hose pipes are at present made from flax fibre but there have been many attempts spread over a large number of years to produce satisfactory unlined hose pipes from ramie fibre in view of the extra strength thus obtainable. The serious disadvantage of the hose pipes produced, however, has been the fact that the water has percolated or leaked through the walls thereof at a relatively rapid rate. Attempts have been made to overcome this latter difficulty by increasing the closeness of the weave but the limitations imposed by the nature of the ramie yarn hitherto available have always precluded the production of a satisfactory hose pipe. It has now been found that the primary cause of the troubles experienced both in hose pipes and in other articles produced from ramie yarn is traceable to the method of production of the yarn itself which has been spun wet.

Ramie fibre cannot be spun into really satisfactory yarn unless it is first sufficiently degummed. This is because the fibres cling together due to the gum remaining and thus cannot be properly combed or otherwise treated to cause them to be arranged straight and parallel in which processes they then break.

The treatment of ramie as heretofore carried out has resulted in the gums being only partially removed and the fibres not being completely separated so that the material produced could not be satisfactorily spun in a dry state; further a large amount of waste was produced in combing. The fibre has therefore been spun in a wet state with the resulting disadvantage that the fibres harden when they become dry and are not suitable for the production of many articles. Thus a hose pipe woven from such fibres will not prevent percolation and leakage of water therethrough. Various methods have been suggested for treating ramie to remove the gums and it has been stated that complete degumming has thus been effected despite the fact that the "degummed"

fibre was harsh and dry and had to be prepared with softening agents in order that it might lend itself easily to the following operations. I have discovered, however, that complete degumming has not heretofore been effected and that in fact it is a difficult matter. If, however, sufficient degumming is effected (i. e. so that not more than 2% of the originally contained gum remains) I have found that the resulting fibre is strong and white and silky in appearance and need not thereafter be subjected as in a prior proposal to treatment to bleach it or to any softening treatment. As would be expected endeavours have been made to spin ramie fibre, degummed to the extent known heretofore, in a dry state, but the yarn produced has been unsatisfactory even when a damping roller was employed on the dry spinning frame. Thus, the best known process for preparing ramie yarn consists in treating the ramie to effect degumming to the extent then possible, taking up the "degummed" fibre on a cylinder to form a lap, cutting the lap into sheets about 10" long, placing the sheets in the "books" of the dressing frame, and then combing and subsequently spinning the fibres. This process inevitably leads to the wastage of many long fibres which are cut into short lengths and cannot in any case produce yarn having the fine count and the soft silky feel, as described herein, which I consider necessary for the production of fire hose or other water-impervious material. It has now been found that by treating the ramie to remove sufficient of the gums i. e. so that not more than 2%, or even less, of the originally contained gum remains as for example by the process described in the specifications of applications Nos. 342,363 and 342,364, yarns may be produced in relatively fine counts and the fibres remain soft and strong. They may also be combed or otherwise treated to cause them to be arranged straight and parallel or substantially so and spun in a dry condition so avoiding the disadvantages of ramie fibres produced as heretofore. This process renders unnecessary the step of taking up on to a cylinder to form a lap and avoids the wastage arising from cutting the lap into narrow sheets for further treatment. The spun yarn may be woven more closely than the ramie yarns so far available and the articles produced have the desirable soft "feel" and effect. An important advantage is that, for instance hose pipes or cloth for making tents may be woven from the yarn with a much closer weave than has hitherto been possible and in this way such articles may be produced which

are better than those at present made from flax fibre.

According to the present invention, ramie yarn to be employed in the production of woven articles, e. g. hose pipes, is produced by a method which consists in treating ramie fibres to effect degumming so that not more than 2% of the originally contained gum remains, then to cause them to be arranged straight and parallel, or substantially so, as for example by combing and then spinning said fibres in the dry state.

The degumming may be satisfactorily effected, for example, by the processes described in my applications Nos. 342,363 and 342,364. It may particularly well be effected if the methods described in both of said applications are used, in which case, in my preferred practice, the ramie fibre is boiled in batches of 50 lbs. in 25 gallons of a solution of a caustic alkali of a concentration of not more than 0.5%, and preferably 0.25%, by weight of caustic alkali, the boiling is continued for not more than half an hour, the treatment medium is drained off, the fibres are squeezed by direct pressure (in contradistinction to centrifugal pressure) to remove the treatment medium and are washed with water which is removed and then neutralized with a weak acid solution e. g. 0.25% hydrochloric acid, and rinsed again, the whole process being repeated at least six times.

The fibres should be separate from each other, i. e. not adhering together and long fibres of at least three inches in length give a particularly satisfactory result.

A further feature of the invention consists in a hose pipe woven from ramie fibre in which the fibre has been treated to cause it to absorb a relatively small proportion of a water-insoluble substance or substances that will prevent deterioration of the fibre. The fibre may be treated to produce the desired result at any desired stage, for example while still in the form of "filasse" (i. e. unspun cleaned fibres), while in the form of yarn or after the pipe has been woven. Suitable substances are various types of wax, with or without appropriate plasticising agents, which are dissolved in a solvent, such as an oil or turpentine, that is later removed and recovered. A certain degree of absorbency is required in the ramie fibre for the proper functioning of the hose pipe produced therefrom and for this reason rubber latex cannot be employed as the treating substance. It is of course known to line canvas hose pipes with rubber but the hose pipes according to the present invention are distinct from such lined pipes.

Alternatively the treatment may be with an emulsion in which the disperse phase is a solution of paraffin wax, for example in turpentine oil and the continuous phase an aqueous solution of a soap containing a very small percentage of alkali, for example, saponified olive oil. If desired, a small proportion of gold size may be added to the emulsion as a drying agent.

The material is heated with the emulsion for a few minutes and the emulsion is then run off. The fibre is squeezed and dried. This treatment may take place in the container in which the degumming treatment described in the specification of application No. 342,363 is effected. The emulsion treatment provides a lubricant on the fibres. After drying, the fibres are combed or

otherwise treated to cause them to be arranged straight and parallel and are then ready for spinning in a dry state.

If the fibre is not thoroughly degummed the 5 yarn is inclined to be wirey, i. e. to have fibre ends projecting from it, which may make it difficult to weave. The friction produced by the projecting ends may cause a tendency for the yarn to fray thereby producing an unsatisfactory result. If 10 the fibre is properly degummed a smoother yarn is produced from which better results are obtained.

It may be noted that the figure of 2% of the 15 natural content of gum resins, to which, at least, the gums contained in the ramie fibre by my process are reduced, is not a critical figure in the sense that products whose gum content are respectively fractionally above and fractionally below 2% differ radically from each other in their 20 properties. There is a more or less progressive improvement in these properties from somewhat above 2% to considerably less than that figure, in respect of the properties which I desire, softness, natural whiteness, ability to comb the fibre 25 without substantial loss into condition for dry-spinning, etc. The figure of 2% is, however, in accordance with my invention, considered as being substantially the upper limit of gum content with which the advantages of my invention may 30 be obtained substantially in commercial practice. In my experience and knowledge of ramie fibre or yarn heretofore produced the gum content has always been 3% and upwards of the natural content of the material, often I should say, 5% and 35 upwards, and it is easily demonstrable that ramie containing such proportions of gum is markedly different, in the properties referred to above, from ramie containing 2% or less, so that the former cannot be used to practise the invention herein 40 described. The figure of 2% is therefore considered critical in the sense described.

It may be stated that ramie ribbons (the raw 45 material) normally contain about 55% by weight of gums. Therefore about 2% of the originally contained gums is also about 2% of the fibre treated by the present process.

What I claim is:

1. A process for the production of ramie yarn 50 for use in preparing woven articles, which consists in repeatedly subjecting ramie fibres to alkali boiling, pressing, and washing to effect sufficient degumming so that not more than 2% of the originally contained gum remains and the treated fibres have a soft feel and a sufficiently 55 white colour to render subsequent bleaching unnecessary, then combing the treated fibres to cause them to be arranged substantially straight and parallel and then spinning them in the dry state.

60 2. A process for the production of ramie yarn for use in preparing woven articles, which consists in repeatedly subjecting ramie fibres to alkali boiling, pressing, and washing to effect sufficient degumming so that not more than 2% 65 of the originally contained gum remains and the treated fibres have a soft feel and a sufficiently white colour to render subsequent bleaching unnecessary, impregnating the fibres with a waxy material, combing them to cause them to be arranged substantially straight and parallel, and then spinning them in the dry state.

MARK SABNER.